

# United States Patent [19]

Tanaka et al.

[11] Patent Number: 4,812,176

[45] Date of Patent: Mar. 14, 1989

[54] PROCESS FOR THE PRODUCTION OF A STRIP OF A CHROMIUM STAINLESS STEEL OF A DUPLEX STRUCTURE HAVING HIGH STRENGTH AND ELONGATION AS WELL AS REDUCED PLANE ANISOTROPY

[75] Inventors: Teruo Tanaka; Katsuhisa Miyakusu; Hiroshi Fujimoto, all of Yamaguchi, Japan

[73] Assignee: Nissin Steel Co., Ltd., Tokyo, Japan

[21] Appl. No.: 134,874

[22] Filed: Dec. 18, 1987

## [30] Foreign Application Priority Data

Dec. 30, 1986 [JP] Japan 61-311959

Dec. 30, 1986 [JP] Japan 61-311960

Jan. 3, 1987 [JP] Japan 62-100

[51] Int. Cl.<sup>4</sup> C21D 8/02

[52] U.S. Cl. 148/12 EA; 148/12 E

[58] Field of Search 148/12 EA, 12 E, 12 C,

148/325

[56]

## References Cited

### U.S. PATENT DOCUMENTS

3,650,848 3/1972 Schneider et al. 148/12 EA

### FOREIGN PATENT DOCUMENTS

2023657 1/1980 United Kingdom 148/325

Primary Examiner—Deborah Yee

Attorney, Agent, or Firm—Wenderoth, Lind & Ponack

[57]

## ABSTRACT

Process for producing steel strip of duplex structure wherein cold rolled strip of chromium stainless steel comprising, in addition to Fe, 10.0% to 20.0% of Cr, to 0.15% of C, to 0.12% of N, the (C+N) being 0.02% to 0.20%, to 2.0% of Si, to 1.0% of Mn and to 0.6% of Ni, is continuously passed through a heating zone where it is heated to form a two-phase of ferrite and austenite and the heated strip is cooled at a cooling rate sufficient to transform the austenite to martensite. The product has high strength and elongation reduced plane anisotropy and hardness of at least HV 200.

11 Claims, 6 Drawing Sheets



FIG. 1



FIG. 2



FIG. 3



FIG. 4



100 $\mu$ m

FIG. 5



FIG. 6

100  $\mu\text{m}$

**PROCESS FOR THE PRODUCTION OF A STRIP OF A CHROMIUM STAINLESS STEEL OF A DUPLEX STRUCTURE HAVING HIGH STRENGTH AND ELONGATION AS WELL AS REDUCED PLANE ANISOTROPY**

**FIELD OF THE INVENTION**

The present invention relates to a novel process for the commercial production of a strip of high strength chromium stainless steel of a dual phase structure having excellent elongation as well as reduced plane anisotropy regarding strength and elongation. The product is useful as a material to be formed into shapes, by e.g. press-forming, which are required to have high strength.

**BACKGROUND OF THE FIELD**

Chromium stainless steels containing chromium as a main alloying element are classified into martensitic and ferritic stainless steels. They are inexpensive when compared with austenitic stainless steels containing chromium and nickel as main alloying elements, and have properties, including ferromagnetism and small thermal expansion coefficient, which are not found in austenitic stainless steels. Accordingly, there are many applications in which chromium stainless steels are used not only for economical reasons but also in view of their properties. Particularly, in the field of parts and attachments of electronic instruments and precision machines where chromium stainless steel sheets are used, as the demand is increasing in recent years, requirements for high efficiency, miniaturization, integration and high precision of worked products as well as simplification of the working process are becoming more and more severe. Thus, in addition to the corrosion resistance inherent to stainless steels and the above-mentioned properties of chromium stainless steels, chromium stainless sheets as a material for working are required to have still higher strength, better workability and more precision. Accordingly, chromium stainless sheets as a material for working, which have a combination of high strength and high elongation conflicting each other, and which are excellent in thickness precision before working and in shape precision after working, are desired in the art.

**PRIOR ART**

Regarding the strength of conventional chromium stainless steel sheet materials, it is well-known that martensitic stainless steels have great strength. For example, 7 species of martensitic stainless steel are prescribed in JIS G 4305 relating to cold rolled stainless steel sheets. The carbon content of these martensitic stainless steels range from up to 0.08% (for SUS410S) to 0.60-0.75% (for SUS440A). They contain higher C when compared with ferritic stainless steels of the same Cr level, and high strength can be imparted to by quenching treatment or by quenching and tempering treatment. For example, it is disclosed in JIS G 4305 that SUS420J2 containing 0.26-0.40% of C and 12.00-14.00% of Cr hardens to at least HRC 40 by quenching from 980°-1040° C. followed by tempering (heating at 150°-400° C. and allowing to cool in air), and that SUS440A containing 0.60-0.75% of C and 16.00-18.00% of Cr also hardens to at least HRC 40 by

quenching from 1010°-1070° C. followed by tempering (heating at 150°-400° C. and allowing to cool in air).

On the other hand with ferritic stainless steel sheets of chromium stainless steel, hardening by heat-treatment is not so much expected, and therefore, it is practiced to increase the strength by work hardening. The method comprises annealing and cold temper rolling. However, the fact is such that ferritic stainless steels are not attractive in applications where high strength is required.

**PROBLEMS**

In the quenched or quenched and tempered condition, martensitic stainless sheets have basically martensitic structure, and have great strength and hardness. But elongation is extremely poor in that condition. Accordingly, once quenched or quenched and tempered, subsequent working or forming is very difficult. In particular, working or forming such as press-forming is impossible after quenching or after quenching and tempering. Accordingly, any working or forming is carried out prior to quenching or quenching and tempering treatment. Usually, a steel maker delivers the material in the annealed condition, that is in a soft condition of low strength and hardness as shown in Table 16 of JIS G 4305 to a working or forming processor, where the material is worked or formed to a shape approximate to that of the final product and thereafter subjected to quenching or quenching and tempering treatment. In many cases surface oxide film or scale formed by the quenching or quenching and tempering treatment is undesirable with stainless steels where surface prettiness is important. Thus, It becomes necessary for the working or forming processor to carry out the heat-treatment of the shaped final product in vacuum or in an inert gas atmosphere or to remove scale from the shaped product. The burden of heat-treatment at the processor side necessarily increases the cost of the product.

Ferritic stainless steel sheets whose strength has been increased by temper rolling have poor workability because of their poor strength-elongation balance due to the elongation markedly reduced by the temper rolling. Further, temper rolling increases the proof stress of the material rather than the tensile strength thereof. In consequence, with a material temper rolled at a high reduction rate, a difference between the proof stress and tensile strength becomes small, and the yield ratio (a ratio of proof stress to tensile strength) approaches 1, rendering the plastic workable range of the material narrow. Generally, a material of high proof stress does not have a good shape after forming such as press-forming because of its great spring-back. Moreover, a temper rolled material exhibits significantly prominent plane anisotropy regarding strength and elongation. Because of these reasons a temper rolled material is not necessarily formed to a good shape even by slight press-forming. Further, as is known, when a steel sheet is rolled, the nearer the surfaces of the sheet the greater the strain. Thus, a temper rolled material inevitably poses a problem of a non-uniform distribution of strain in a direction of thickness, and in turn non-uniform distribution of residual stress in a direction of thickness, which can be a cause of a shape distortion, such as a warp of sheet, appearing in ultra-thin sheets after they have been subjected to forming holes by a photo-etching process or to blanking. The shape distortion is serious in applications, such as electronic parts, where high precision is required. In addition to the above-mentioned problems

relating to their properties, temper rolled materials pose many other problems relating to the management of their manufacture. Regarding control of the strength, since work hardening by cold rolling is utilized in temper rolling, the reduction rate is the most important factor determining the strength. Accordingly, in order that products of desired thickness and strength are precisely and stably produced, severe control of the reduction rate as well as severe control of the initial thickness and strength of the material prior to temper rolling is necessary. Regarding control of the shape, cold rolling of a reduction rate of several tens % is contemplated here where increase of strength is aimed, different from skin-pass rolling or other rolling of a reduction rate of at most 2 or 3% where rectification of shape is aimed. By cold rolling of a reduction rate of several tens % it is difficult to provide a product having a precise shape in the cold rolled condition. It is often necessary, therefore, to subject the as cold rolled material to a treatment for the removal of stress, in which the material is heated, for the purpose of the rectification of the shape, to a temperature which is lower than the recovery-recrystallization temperature of the material and at which the material is not softened.

In addition to the above-discussed problems owing to temper rolling, ferritic stainless steel sheets involve a problem of ridging, which may be said inherent thereto. While a ridging is a kind of surface defects normally formed on surfaces of a cold rolled and annealed sheet of a ferritic stainless sheet when it is press-formed, surface defects called cold rolling ridges are frequently found on surfaces of a temper rolled sheet of a ferritic stainless steel. Formation of such ridges is a serious problem in applications where surface flatness is important.

#### Measures to Solve the Problems

The problems noted above will be solved, if a chromium stainless steel having moderately high strength, good elongation and formability enabling the steel to be formed into a desired shape, reduced anisotropy and no problems of ridging will be provided in the form of a strip at the side of a steel maker. For this purpose, an extensive research work on chromium stainless steels has been carried out in both the aspects of the steel composition and the manufacturing process. As a result, it has now been found that substantially all of the above-mentioned problems are successfully solved by a process according to the invention for the production of a strip of a chromium stainless steel of a duplex structure, consisting essentially of ferrite and martensite, having high strength and elongation as well as reduced plane anisotropy and having a hardness of at least HV 200, which process comprises:

a step of hot rolling a slab of a steel to provide a hot rolled strip, said steel comprising, by weight, in addition to Fe, from 10.0% to 20.0% of Cr, up to 0.15% of C, up to 0.12% of N, the (C+N) being not less than 0.02% but not more than 0.20%, up to 2.0% of Si, up to 1.0% of Mn and up to 0.6% of Ni;

a step of cold rolling the hot rolled strip to provide a cold rolled strip of a desired thickness, with preference to at least two steps of cold rolling to provide a cold rolled strip of a desired thickness, including a step of intermediate annealing between the successive two cold rolling steps, said intermediate annealing comprising heating and maintaining the strip at a temperature to form a single phase of ferrite; and

a step of continuous finish heat treatment in which the cold rolled strip is continuously passed through a heating zone where it is heated to a temperature ranging from the  $Ac_1$  point of the steel to 1100° C. to form a two-phase of ferrite and austenite and maintained at that temperature for not longer than 10 minutes, and the heated strip is cooled at a cooling rate sufficient to transform the austenite to martensite.

The invention not only solves the above-mentioned problems, but also provides a novel commercial process for the production of a strip of a chromium stainless steel. The process of the invention is advantageous in that the strength of the product can be freely and simply adjusted by controlling the steel composition, the heating temperature in the finish heat treatment, and/or the cooling rate in the finish heat treatment. The product of the process of the invention has a combination of strength and elongation which is not seen in commercially available martensitic or ferritic stainless steel strips, and exhibits reduced plane anisotropy regarding strength and elongation. The product of the invention is delivered to the market in the form of a coil of strip.

It was known in the art that when a typical ferritic stainless steel, for example SUS430, is heated to a temperature above the  $Ac_1$  point austenite is formed, and that when the steel so heated is then quenched the austenite is transformed to martensite, resulting in a duplex structure of ferrite and martensite. However, in the production of a cold rolled strip of a ferritic stainless steel capable of forming austenite at a high temperature, any heat treatment of the cold rolled strip has strictly been an annealing at a temperature under which a single phase of ferrite is stable. A heat treatment of the cold rolled strip at a temperature high enough to eventually form martensite has been commonly avoided as bringing about deterioration of quality such as elongation, and has been ignored in the commercial production of strips. Accordingly, so far as we know, there are no patents and metallurgical literatures in which a continuous heat treatment of a cold rolled strip of a chromium stainless steel is considered as in the invention, and in which on chromium stainless steel strips which have undergone a finish heat treatment comprising heating the cold rolled strip to a temperature high enough to form a two-phase of ferrite and austemite, the relationship between the tensile behavior and the heating temperature as well as the anisotropy regarding the strength and elongation are studied in detail. The invention provides a novel commercial process for the production of a high strength chromium stainless steel strip, and also provides, as a result, a novel chromium stainless steel material in the form of a strip having excellent properties which have not been possessed by conventional strips of chromium stainless steels.

#### DETAILED DESCRIPTION OF THE INVENTION

The invention will now be described in detail, in particular, regarding the chemical composition of the steel and the steps and conditions of the manufacturing process.

The steel employed in the process of the invention comprises, by weight, in addition to Fe, from 10.0% to 20.0% of Cr, up to 0.15% of C, up to 0.12% of N, the (C+N) being not less than 0.02% but not more than 0.20%, up to 2.0% of Si, up to 1.0% of Mn and up to 0.6% of Ni.

Cr must be contained in an amount of at least 10.0% to achieve the desired level of corrosion resistance as stainless steels. However, as the Cr content increases, the amounts of austenite formers required for eventual formation of martensite to achieve high strength on the one hand, and the product becomes expensive on the other hand. Accordingly, the upper limit for Cr is now set as 20.0%. Chromium stainless steels containing up to 14.0% of Cr will be referred to herein as low Cr steels, while chromium stainless steels containing Cr in excess of 14.0% as high Cr steels.

C and N are strong and inexpensive austenite formers when compared with Ni and Mn and have an ability of greatly strengthening martensite. Accordingly, they are effective to control and increase the strength of the product. The permissible lower limit for (C+N) depends upon the particular Cr content and the particular amount of other austenite formers. For low chromium steels at least 0.02% of (C+N) is required to obtain a product of a duplex structure containing a substantial amount of martensite and having a hardness of at least HV200. As the Cr content increases the minimum amount of (C+N) required increases. Thus, at least 0.03% of (C+N) will be required, although depending upon the particular contents of Mn and Ni. On the other hand an excessively high content of (C+N) should be avoided, or otherwise the amount of martensite eventually formed increases, often to 100%, and the hardness of the formed martensite phase itself becomes unduly high, rendering the elongation of the product poor. The upper limit for (C+N) depends upon the particular Cr content. For low Cr steels (C+N) should be controlled not more than 0.12%. Whereas in steels of relatively high Cr (more than 14.0% of Cr) the (C+N) content up to 0.20% is permissible.

C is controlled at a level of not more than 0.15%, and in particular not more than 0.10% for low Cr steels. If C is excessively high, the corrosion resistance of the product may be impaired, due to precipitation of Cr carbide in grain boundaries during the cooling step of 40 the continuous heat treatment.

The upper limit for N depends upon the chromium content. For steels of a relatively high Cr, N may be up to 0.12%. Whereas for low Cr steels, N should preferably be controlled not in excess of 0.08%. The presence 45 of an unduly high amount of N may be a cause of increase of surface defects.

Si is a ferrite former and acts to dissolve in both the ferritic and martensitic phases thereby to strengthen the product. The upper limit for Si is set as 2.0%, since the 50 presence of an excessively high amount of Si adversely affects the hot and cold workabilities of the product.

Mn and Ni are austenite formers and are useful for the control of the amount of martensite and the strength of the product. For economical reasons the upper limits 55 for these elements are set as 1.0% for Mn and 0.6% for Ni, respectively, as normally allowed for standardized chromium ferritic and martensitic steels.

In addition to the above-mentioned alloying elements, the steel of the invention may optionally contain 60 at least one other useful element selected from up to 0.20% of Al, up to 0.0050% of B, up to 2.5% of Mo, up to 0.10% of REM (rare earth metals) and up to 0.20% of Y.

A1 is an element effective for deoxygenation and 65 serves to remarkably reduce A2 inclusions which adversely affect press formability of the product. However, as the A1 content approaches and exceeds 0.20%,

such an effect of A1 becomes saturated on the one hand, surface defects tend to increase. Accordingly, the upper limit for A1 is now set as 0.20%.

B is effective for improving the toughness of the product. While such an effect may be realized even with a trace of B, it becomes saturated as B approaches and exceeds 0.0050%. For this reason we set the upper limit for B as 0.0050%.

Mo is effective for enhancing corrosion resistance of the product. For an economical reason the upper for Mo is set as 2.5%.

REM and Y are effective for enhancing hot workability and oxidation resistance at a high temperature. They effectively serve to suppress formation of oxide scales during the continuous finish heat treatment carried out according to the invention at a high temperature thereby to provide a good surface texture after descaling. These effects tend to be saturated, however, as REM and Y approach and exceed 0.10% and 0.20%, respectively. Accordingly, the upper limits for REM and Y are now set as 0.10% for REM and 0.20% for Y, respectively.

Besides the above-mentioned useful alloying elements, the steel of the invention may contain residual amounts of S, P, and O.

As to S, the less the more preferable, since it is harmful to corrosion resistance and hot workability of the steel. The upper limit for S is now set as 0.030%.

P serves to strengthen the steel by dissolving therein. However, we set the upper limit for P as 0.040%, as prescribed in standards of conventional ferritic and martensitic steels, since P may adversely affect toughness of the product.

O forms non-metallic inclusions, and thereby impairs purity of the steel. For this reason the upper limit for O is set as 0.02%.

Thus, according to one embodiment of the invention the steel employed consists essentially of, by weight,:

up to 0.10% of C,  
up to 2.0% of Si,  
up to 1.0% of Mn,  
up to 0.040% of P,  
up to 0.030% of S,  
up to 0.60% of Ni,  
from 10.0% to 14.0% of Cr,  
up to 0.08% of N, the (C+N) being not less than 0.02% but not more than 0.12%,  
up to 0.02% of O, and optionally at least one element selected from the group consisting of:  
up to 0.20% of Al,  
up to 0.0050% of B,  
up to 2.5% of Mo,  
up to 0.10% of REM and  
up to 0.20% of Y, the balance being Fe and unavoidable impurities.

In accordance with another embodiment of the invention, the steel employed consists essentially of, by weight,:

up to 0.15% of C,  
up to 2.0% of Si,  
up to 1.0% of Mn,  
up to 0.040% of P,  
up to 0.030% of S,  
up to 0.60% of Ni,  
more than 14.0% to 20.0% of Cr,  
up to 0.12% of N, the (C+N) being not less than 0.03% but not more than 0.20%,

up to 0.02% of O, and optionally at least one element selected from the group consisting of:  
 up to 0.20% of A1,  
 up to 0.0050% of B,  
 up to 2.5% of Mo,  
 up to 0.10% of REM and  
 up to 0.20% of Y, the balance being Fe and unavoidable impurities.

The process according to the invention comprises the steps of hot rolling, cold rolling and continuous finish heat treatment.

#### Hot Rolling

A slab of a chromium stainless steel having a selected chemical composition, which has been prepared by a conventional steel making and casting technique, is hot rolled to provide a hot rolled strip by a conventional technique. For example, the hot rolling is started at a temperature of about 1100° C. to 1200° C. and ends at a temperature of about 850° C. The hot rolled strip is then coiled at a temperature of about 650° C., and the coil normally having a weight of from about 8 to about 15 tons is allowed to cool in air. The cooling rate of such a coil is very slow. On the other hand, although the chromium stainless steel employed has a two-phase structure of austenite and ferrite at high temperatures at which it is hot rolled, a rate of transformation from the austenite to ferrite caused by temperature decrease is slower with the chromium stainless steel than with low carbon steels. Thus, in the strip of the invention as hot rolled those portions of the steel which were austenite at the high temperatures have not completely been transformed to ferrite. The steel of the invention in the hot rolled condition has a stratified band-like structure of a phase which comprises intermediates of the transformation from the austenite to ferrite, such as bainite, and a phase which has been the ferrite, both the phases being more or less elongated in the direction of hot rolling. The hot rolled strip is preferably annealed and descaled. The annealing of the hot rolled strip not only softens the material to enhance the cold rollability of the hot rolled strip, but also transforms and decomposes, to some extent, the above-mentioned intermediate transformed phase (which were austenite at the high temperatures of the hot rolling) in the as hot rolled strip to ferrite and carbides. Either continuous annealing or box annealing may be applied for annealing the hot rolled strip.

#### Cold Rolling

The hot rolled strip, preferably after annealed and descaled, is cold rolled to a desired thickness, which can be as thin as from about 0.1 mm to about 1.0 mm in cases wherein the product of the invention is intended to be used as a material for the fabrication of parts of electronic instruments and precision machines by press-forming.

The cold rolling may be carried out in a single step of cold rolling with no intermediate annealing. By the expression "a single step of cold rolling with no intermediate annealing", we mean to reduce the thickness of the strip from that of the hot rolled strip to a desired one of the cold rolled strip either by one-pass cold rolling or by multiple-pass cold rolling without any intermediate annealing, irrespective of the number of passes through rollers. The rolling rate of reduction in thickness may range from about 30% to about 95%. The product which has been cold rolled in a single step of cold roll-

ing with no intermediate annealing, and thereafter finish heat treated will be referred to herein as a 1CR material.

Preferably, the cold rolling is carried out in at least two steps of cold rolling, including a step of intermediate annealing between the two successive cold rolling steps. The intermediate annealing comprises heating the cold rolled strip to a temperature at which a single phase of ferrite may be formed prior to the subsequent cold rolling. Apparently, the temperature for the intermediate annealing is below the Ac1 Point of the steel. In each cold rolling step the thickness of the strip is reduced by passing the strip, at least once, through rollers. The reduction rate in each cold rolling step is preferably at least about 30%. The product, which has been cold rolled in at least two steps of cold rolling with a step of intermediate annealing between the successive two cold rolling steps, and thereafter finish heat treated, will be referred to herein as a 2CR material. While 1CR materials have satisfactorily reduced plane anisotropy in respect of strength and elongation, the corresponding 2CR materials exhibit further reduced plane anisotropy.

The cold rolling is essential for the purposes of the invention. When the hot rolled strip, as such or after annealing, is subjected to the continuous finish heat treatment described herein, a two-phase structure of ferrite and martensite is basically realized. The structure obtained, however, more or less succeeds to that of the hot rolled strip, and comprises relatively large grains of ferrite and martensite aligned, respectively, in the direction of rolling, resulting in significant plane anisotropy in respect of strength and elongation. In contrast, when the hot rolled strip, preferably after annealing, is cold rolled, preferably in at least two steps with a step of intermediate annealing comprising heating the strip to a temperature to form a single phase of ferrite between the successive two cold rolling steps, and then subjected to the continuous finish heat treatment according to the invention, the stratified band-like structure of the steel in the hot rolled condition collapses and a duplex structure of uniformly admixed fine ferrite and martensite is obtained. Thus, the product of the invention exhibits reduced plane anisotropy in respect of strength and elongation, and has excellent workability or formability. Further, without cold rolling it is very difficult to prepare thin steel strips which meet severe requirements for thickness precision, shape precision and surface qualities.

#### Continuous Finish Heat Treatment

50 The cold rolled strip is continuously passed through a heating zone where it is heated to a temperature ranging from the Ac1 point of the steel to 1100° C. to form a two-phase of ferrite and austenite and maintained at that temperature for not longer than 10 minutes, and the heated strip is cooled at a cooling rate sufficient to transform the austenite to martensite.

In the continuous finish heat treatment according to the invention, it is essential to heat the cold rolled strip to a temperature at which a two-phase of ferrite and austenite may be formed, that is to a temperature not lower than Ac1 point of the steel. However, in a continuous heat treatment using a temperature near the Ac1 point of the steel, the amount of austenite formed significantly varies with a slight change of the temperature, and in consequence there is frequently a case wherein a desired level of hardness is not stably obtained after quenching. We have found that such undesirable variations of hardness can be avoided if a heating tempera-

ture of at least about 100° C. above the  $Ac_1$  point of the steel is used. Thus, a preferable heating temperature in the continuous heat treatment of the invention is at least about 100° C. above the  $Ac_1$  point of the steel, more specifically, at least about 900° C., and more preferably, at least about 950° C. The upper limit for the heating temperature is not very critical. Generally, the higher the temperature, the more the steel is strengthened. However, as the heating temperature approaches 1100° C., the strengthening effect becomes saturated or occasionally even decreased, and the energy consumption is increased. Accordingly, we set the upper limit for the heating temperature as about 1100° C.

As to metallurgical significances of the heating of the cold rolled strip to a temperature at which a two-phase structure of ferrite and austenite is formed, we can men-

products upon the heating temperature in the finish heat treatment;

FIG. 4 is a photo showing a metallic structure of a low Cr 2CR product;

5 FIG. 5 is a graph showing the dependence of the amount of martensite and the hardness of high Cr 2CR products upon the heating temperature in the finish heat treatment; and

10 FIG. 6 is a photo showing a metallic structure of a high Cr 2CR product.

#### EXAMPLE 1

This example relates to experiments demonstrating the dependence of the amount of martensite and the hardness of 1CR products upon the heating temperature in the finish heat treatment

TABLE 1

| Steel | C     | Si   | Mn   | P     | S     | Ni   | (in % by weight) |       |        |       |
|-------|-------|------|------|-------|-------|------|------------------|-------|--------|-------|
|       |       |      |      |       |       |      | Cr               | N     | Al     | O     |
| A     | 0.040 | 0.18 | 0.20 | 0.021 | 0.010 | 0.10 | 11.94            | 0.035 | 0.018  | 0.008 |
| B     | 0.102 | 0.45 | 0.76 | 0.020 | 0.009 | 0.10 | 17.25            | 0.026 | <0.005 | 0.012 |
| C     | 0.068 | 0.46 | 0.40 | 0.018 | 0.008 | 0.09 | 16.44            | 0.022 | <0.005 | 0.018 |

tion dissolution of Cr carbide and nitride, formation of austenite and concentration of C and N into the formed austenite. For the steels concerned here, these phenomena reach equilibrium within a short period of time. Accordingly, the heating time for which the material being treated is maintained at the required temperature can be as short as not more than about 10 minutes. This shortness of the heating time renders the process of the invention advantageous from view points of production efficiency and manufacturing costs. By the above-mentioned heating conditions it is possible to form an amount of austenite sufficient to eventually provide at 35 least about 10% (in case of high Cr steels) or at least about 20% (in cases of low Cr steels) by volume of martensite.

The cooling rate in the continuous finish heat treatment should be sufficient to transform the austenite to martensite. Practically, a cooling rate of at least about 1° C./sec, preferably at least about 5° C./sec may be used. The upper limit for the cooling rate is not critical but a cooling rate in excess of about 500° C. will not be practical. The cooling rate prescribed above is maintained until the austenite has been transformed to martensite. It should be appreciated that after the transformation has been completed the cooling rate is not critical. The cooling of the strip may be carried out either by application of a gaseous or liquid cooling medium to the strip or by roll cooling using water-cooled rolls. It is convenient to carry out the continuous heat treatment of the cold rolled strip according to the invention by continuously uncoiling a coil of the cold rolled strip, passing it through a continuous heat treatment furnace having heating and quenching zones, and coiling the treated strip.

The invention will be further described by the following Examples with reference to the attached drawings in which

FIG. 1 is a graph showing the dependence of the amount of martensite and the hardness of 1CR products upon the heating temperature in the finish heat treatment;

FIG. 2 is a photo showing a metallic structure of a 65 1CR product;

FIG. 3 is a graph showing the dependence of the amount of martensite and the hardness of low Cr 2CR

25

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 923

## EXAMPLE 2

This example relates to experiments demonstrating properties of a 1CR material of a duplex structure compared with those of a temper rolled material of the same chemical composition. The tested materials were prepared by the processes as noted below.

## (1). 1CR material

A hot rolled sheet of Steel B of a thickness of 3.6 mm was annealed at a temperature of 780° C. for 6 hours in a furnace, allowed to cool in the same furnace, pickled, cold rolled to a thickness of 0.7 mm (a reduction rate of 80.6%) in a single step of cold rolling with no intermediate annealing, heated at a temperature of 970° C. for about 1 minute and cooled at an average cooling rate of about 20° C./sec. to ambient temperature. FIG. 2 is a photo showing the metallic structure of the material so prepared. In the photo, areas appearing white are ferrite, while areas appearing dark or grey are martensite. It can be seen that the material has a duplex structure of uniformly admixed fine ferrite and martensite grains.

## (2). Temper rolled material

A hot rolled sheet of Steel B of a thickness of 3.6 mm was annealed at a temperature of 780° for 6 hours in a furnace and allowed to cool in the same furnace, pickled, cold rolled to a thickness of 2.0 mm, annealed at a temperature of 800° C. for 1 minute, air cooled, and temper rolled to a thickness of 0.7 mm.

Specimens of both the materials were tested for tensile strength (kgf/mm<sup>2</sup>) and elongation (%) in directions of, 0° (L), 45° (D) and 90° (T) to the rolling direction, as well as hardness. The results are shown in Table 2 below.

TABLE 2

| Process | Hardness (HV) | Tensile strength (kgf/mm <sup>2</sup> ) |      |       | Elongation (%) |      |     |
|---------|---------------|-----------------------------------------|------|-------|----------------|------|-----|
|         |               | L                                       | D    | T     | L              | D    | T   |
| (1)     | 288           | 94.7                                    | 90.0 | 95.8  | 10.2           | 12.8 | 8.4 |
| (2)     | 280           | 91.1                                    | 97.2 | 108.5 | 2.7            | 1.8  | 0.9 |

(1). 1CR material of a duplex structure finish heat treated at 970° C.

(2). Temper rolled material temper rolled at a reduction rate of 65%

Table 2 reveals that the 1CR material of a duplex structure has remarkably high elongation in all directions when compared with the temper rolled material of the same chemical composition having the same level of hardness and strength. Table 2 further reveals that the 1CR material of a duplex structure exhibits improved plane isotropy in respect of strength and elongation when compared with the temper rolled material of the same chemical composition having the same level of hardness and strength.

## EXAMPLE 3

This example relates to experiments demonstrating the dependence of the amount of martensite and the hardness of low Cr 2CR products upon the heating temperature in the finish heat treatment

TABLE 3

| Steel | (in % by weight) |      |      |       |       |      |       |       |       |       |
|-------|------------------|------|------|-------|-------|------|-------|-------|-------|-------|
|       | C                | Si   | Mn   | P     | S     | Ni   | Cr    | N     | Al    | O     |
| D     | 0.021            | 0.55 | 0.41 | 0.018 | 0.006 | 0.15 | 12.22 | 0.009 | 0.023 | 0.006 |
| E     | 0.033            | 0.54 | 0.45 | 0.018 | 0.006 | 0.16 | 12.19 | 0.009 | 0.008 | 0.008 |

Steels D and E having chemical compositions indicated in Table 3 and Steel A of Table 1 were cast, hot rolled to a thickness of 3.6 mm, annealed at a temperature of 780° C. for 6 hours in a furnace, allowed to cool in the same furnace, pickled and cold rolled to a thickness of 1.0 mm, annealed at a temperature of 800° C. for 1 minute, air cooled, and cold rolled to a thickness of 0.3 mm. Sheets cut from each cold rolled material were heated at various temperatures ranging from 850° C. to 1080° C. for about 1 minute and cooled at an average cooling rate of about 20° C./sec. to ambient temperature. The amount of martensite (% by volume) and the hardness (HV) of the products were determined. The results are shown in FIG. 3, in which symbols D, E and A designate Steels D, E and A, respectively. The same observations as those here-in-before made on FIG. 1, will be made on FIG. 3.

## EXAMPLE 4

This example relates to experiments demonstrating properties of a low Cr 2CR material of a duplex structure compared with those of 1CR and temper rolled materials of the same chemical composition. The tested materials were prepared by the processes as noted below.

## (3). 2CR material

A hot rolled sheet of Steel E of a thickness of 3.6 mm was annealed at a temperature of 780° C. for 6 hours in a furnace, allowed to cool in the same furnace, pickled, cold rolled to a thickness of 1.0 mm, annealed at a temperature of about 800° C. for 1 minute, air cooled and cold rolled to a thickness of 0.3 mm. The sheet was heated at a temperature of 980° C. for about 1 minute and cooled at an average cooling rate of about 20° C./sec. to ambient temperature. FIG. 4 is a photo showing the metallic structure of the material so prepared. In the photo, areas appearing white are ferrite, while areas appearing dark or grey are martensite. It can be seen that the material has a duplex structure of uniformly admixed fine ferrite and martensite grains.

## (4). 1CR material

The process (3) above was repeated except that the hot rolled, annealed and pickled sheet was cold rolled to a thickness of 0.3 mm in a single step of cold rolling with no intermediate annealing.

## (5). Temper rolled material

A hot rolled sheet of Steel E of a thickness of 3.6 mm was annealed at a temperature of 780° C. for 6 hours in a furnace, allowed to cool in the same furnace, pickled, cold rolled to a thickness of 1.2 mm, annealed at a temperature of 800° C. for 1 minute and temper rolled to a thickness of 0.3 mm.

Specimens of the materials so prepared were tested for tensile strength (kgf/mm<sup>2</sup>) and elongation (%) in directions of, 0° (L), 45° (D) and 90° (T) to the rolling direction, as well as hardness. The results are shown in Table 4 below.

TABLE 4

| Process | Hardness (HV) | Tensile strength (kgf/mm <sup>2</sup> ) |      |      | Elongation (%) |      |      |
|---------|---------------|-----------------------------------------|------|------|----------------|------|------|
|         |               | L                                       | D    | T    | L              | D    | T    |
| (3)     | 256           | 82.5                                    | 85.1 | 83.8 | 12.5           | 10.8 | 11.8 |
| (4)     | 265           | 88.1                                    | 85.2 | 88.4 | 10.9           | 12.0 | 7.9  |
| (5)     | 265           | 87.3                                    | 93.5 | 97.7 | 2.7            | 1.4  | 0.8  |

(3). 2 CR material of a duplex structure finish heat treated at 980° C.

(4). 1 CR material of a duplex structure finish heat treated at 980° C.

(5). Temper rolled material temper rolled at a reduction rate of 75%

Table 4 reveals that when compared with the temper rolled material of the same chemical composition having the same level of hardness and strength, both the 1CR and 2CR materials of a duplex structure have remarkably high elongation in all directions, and exhibit improved plane isotropy in respect of strength and elongation. Table 4 further reveals the preference of the 2CR material to the 1CR material in view of the further reduced plane anisotropy of the former.

#### EXAMPLE 5

This example relates to experiments demonstrating the dependence of the amount of martensite and the hardness of high Cr 2CR products upon the heating temperature in the finish heat treatment

TABLE 5

| Steel | (in % by weight) |      |      |       |       |      |       |       |        |       |
|-------|------------------|------|------|-------|-------|------|-------|-------|--------|-------|
|       | C                | Si   | Mn   | P     | S     | Ni   | Cr    | N     | Al     | O     |
| F     | 0.068            | 0.46 | 0.40 | 0.018 | 0.008 | 0.09 | 16.44 | 0.022 | <0.005 | 0.018 |
| G     | 0.088            | 0.57 | 0.82 | 0.021 | 0.009 | 0.12 | 15.01 | 0.041 | <0.005 | 0.012 |

Steels F and G having chemical compositions indicated in Table 5 and Steel B of Table 1 were cast, hot rolled to a thickness of 3.6 mm, annealed at a temperature of 780° C. for 6 hours in a furnace, allowed to cool in the same furnace, pickled and cold rolled to a thickness of 1.0 mm, annealed at a temperature of 800° C. for 1 minute, air cooled, and cold rolled to a thickness of 0.3 mm. Sheets cut from each cold rolled material were heated at various temperatures ranging from 800° C. at 1150° C. for about 1 minute and cooled at an average cooling rate of about 20° C./sec. to ambient temperature. The amount of martensite (% by volume) and the hardness (HV) of the products were determined. The results are shown in FIG. 5, in which symbols F, G and B designate Steels F, G and B, respectively. The same observations as those here-in-before made on FIG. 1, will be made on FIG. 5.

#### EXAMPLE 6

This example relates to experiments demonstrating properties of a high Cr 2CR material of a duplex structure compared with those of 1CR and temper rolled materials of the same chemical composition. The tested material were prepared by the processes as noted below.

#### (6). 2CR material

The process (3) above was repeated except that Steel B was used instead of Steel E and that the cold rolled sheet was final heat treated at 970° C. instead of 980° C.

#### (7). 1CR material

The process (4) above was repeated except that Steel B was used instead of Steel E and that the cold rolled sheet was final heat treated at 970° C. instead of 980° C.

#### (8). Temper rolled material

The process (5) above was repeated except that Steel B was used instead of Steel E and that the hot rolled, annealed and pickled sheet was cold rolled to a thickness of 1.07 mm instead of 1.2 mm.

Specimens of the materials so prepared were tested for tensile strength (kgf/mm<sup>2</sup>) and elongation (%) in directions of, 0° (L), 45° (D) and 90° (T) to the rolling direction, as well as hardness. The results are shown in Table 6 below.

TABLE 6

| Process | Hardness (HV) | Tensile strength (kgf/mm <sup>2</sup> ) |      |       | Elongation (%) |      |      |
|---------|---------------|-----------------------------------------|------|-------|----------------|------|------|
|         |               | L                                       | D    | T     | L              | D    | T    |
| (6)     | 280           | 91.4                                    | 92.1 | 91.8  | 11.5           | 12.6 | 10.9 |
| (7)     | 283           | 94.7                                    | 90.0 | 95.8  | 10.6           | 12.3 | 7.4  |
| (8)     | 285           | 91.1                                    | 97.2 | 108.5 | 2.4            | 1.2  | 0.8  |

(6): 2 CR material of a duplex structure finish heat treated at 970° C.

(7): 1 CR material of a duplex structure finish heat treated at 970° C.

(8): Temper rolled material temper rolled at a reduction rate of 72%

Table 6 reveals that when compared with the temper rolled material of the same chemical composition having the same level of hardness and strength, both the 1CR and 2CR materials of a duplex structure have re-

markably high elongation in all directions, and exhibit improved plane isotropy in respect of strength and elongation. Table 4 further reveals the preference of the 2CR material to the 1CR material in view of the further reduced plane anisotropy of the former.

#### EXAMPLE 7-18

These examples illustrate commercial production of 1CR materials according to the invention, using a continuous heat treatment furnace.

Steels having chemical compositions indicated in Table 7 were cast, hot rolled to a thickness of 3.6 mm, annealed at a temperature of 780° C. for 6 hours in a furnace, allowed to cool in the same furnace, pickled and cold rolled to a thickness of 0.7 mm (a reduction rate of 80.6%) in a single step of cold rolling with no intermediate annealing. Each cold rolled strip was continuously finish heat treated in a continuous heat treatment furnace under conditions indicated in Table 8 with a time of uniform heating of 1 minute, except for in Examples 17 and 18. In Example 17 the cold rolled strip was heated in a box furnace with a time of uniform heating of about 6 hours and allowed to cool in the same furnace. In Example 18 a hot rolled strip of Steel 1 of a thickness of 3.6 mm was annealed at a temperature of 780° C. for 6 hours in a furnace, allowed to cool in the same furnace, pickled, cold rolled to a thickness of 2.2 mm, annealed at a temperature of 800° C. for 1 minute, air cooled and temper rolled to a thickness of 0.7 mm. Specimens of the products were tested for 0.2% proof stress, tensile strength and elongation in directions of 0° (longitudinal), 45° (diagonal) and 90° (transverse) to the direction of rolling, and for amount of martensite and hardness. On broken specimens from the tensile test, yes

or no of ridging occurrence was observed. The results are shown in Table 8.

Examples 7-13 are in accordance with the invention, whereas Examples 14-18 are controls.

As seen from Table 8, steel strips of a duplex structure containing from about 30 to about 80% by volume of martensite having a combination of great strength and hardness as well as good elongation were obtained by processes of Examples 7-13 according to the invention. The products of the invention exhibited reduced plane anisotropy in respect of 0.2% proof stress, tensile strength and elongation.

In contrast, Steel 8 used in example 14 had a (C+N) content as low as 0.012%, and in consequence, no martensite was formed by the continuous finish heat treatment. The product of Example 14 had poor strength and hardness.

Steel 9 used in Example 15 had a carbon content of

martensite transformed, exhibiting a combination of high elongation with poor strength and hardness, as was the case in Example 16.

The product of Example 18 was a temper rolled material which had, when compared with the products of the invention, remarkably low elongation, high yield ratio (a ratio of 0.2% proof stress to tensile strength) and prominent plane anisotropy in respect of 0.2% proof stress, tensile strength and elongation. Apparently, such a product is inferior to the products of the invention regarding workability or formability and shape precision after worked or formed.

Table 8 further reveals that broken specimens from the tensile test of Examples 14, 16, 17 and 18 showed occurrence of ridging. In contrast the products of the invention were completely free from the problem of ridging. This means that the products of the invention work well in press forming.

TABLE 7

| Steel | C     | Si   | Mn   | P     | S     | (in % by weight) |       |       |       |       |                    |  |  |
|-------|-------|------|------|-------|-------|------------------|-------|-------|-------|-------|--------------------|--|--|
|       |       |      |      |       |       | Ni               | Cr    | N     | Al    | O     | Others             |  |  |
| 1     | 0.021 | 0.58 | 0.53 | 0.027 | 0.004 | 0.08             | 13.29 | 0.062 | 0.013 | 0.008 |                    |  |  |
| 2     | 0.083 | 0.54 | 0.45 | 0.018 | 0.006 | 0.16             | 12.08 | 0.009 | 0.150 | 0.007 |                    |  |  |
| 3     | 0.116 | 0.41 | 0.60 | 0.022 | 0.006 | 0.12             | 18.21 | 0.013 | 0.018 | 0.008 |                    |  |  |
| 4     | 0.086 | 1.51 | 0.31 | 0.018 | 0.006 | 0.17             | 16.55 | 0.032 | 0.005 | 0.015 |                    |  |  |
| 5     | 0.043 | 0.52 | 0.39 | 0.018 | 0.005 | 0.21             | 13.51 | 0.009 | 0.009 | 0.007 | B 0.0023           |  |  |
| 6     | 0.035 | 0.46 | 0.53 | 0.021 | 0.005 | 0.12             | 16.38 | 0.104 | 0.130 | 0.006 | Mo 0.55            |  |  |
| 7     | 0.075 | 0.45 | 0.51 | 0.018 | 0.001 | 0.12             | 16.48 | 0.028 | 0.018 | 0.010 | REM 0.025, Y 0.031 |  |  |
| 8     | 0.006 | 0.47 | 0.29 | 0.020 | 0.006 | 0.11             | 16.21 | 0.006 | 0.010 | 0.009 |                    |  |  |
| 9     | 0.155 | 0.63 | 0.45 | 0.021 | 0.005 | 0.10             | 14.31 | 0.065 | 0.027 | 0.015 |                    |  |  |

TABLE 8

| Ex. | St. | Finish heat treatment |      |                 | Amount of martensite (% by vol) | 0.2% proof (kgf/mm <sup>2</sup> ) |       |       | Properties (3) |       |      | Hardness | ridging |     |     |  |
|-----|-----|-----------------------|------|-----------------|---------------------------------|-----------------------------------|-------|-------|----------------|-------|------|----------|---------|-----|-----|--|
|     |     | (1)                   | (2)  | temperature °C. |                                 | L                                 | D     | T     | L              | D     | T    |          |         |     |     |  |
|     |     |                       |      |                 |                                 |                                   |       |       |                |       |      |          |         |     |     |  |
| 7   | 1   | 1000                  | 250  | 78.5            | 69.4                            | 69.1                              | 70.6  | 97.8  | 95.1           | 106.5 | 9.5  | 10.1     | 8.5     | 313 | No  |  |
| 8   | 2   | 980                   | 35   | 67.5            | 57.2                            | 54.3                              | 59.1  | 83.1  | 81.8           | 88.4  | 11.2 | 13.8     | 8.7     | 265 | No  |  |
| 9   | 3   | 940                   | 15   | 39.6            | 48.8                            | 47.0                              | 52.5  | 85.8  | 82.7           | 90.5  | 12.3 | 16.8     | 11.1    | 252 | No  |  |
| 10  | 4   | 1050                  | 175  | 31.5            | 44.5                            | 42.9                              | 45.1  | 90.6  | 87.3           | 89.5  | 12.1 | 15.7     | 11.6    | 247 | No  |  |
| 11  | 5   | 1000                  | 20   | 59.3            | 52.7                            | 50.1                              | 53.6  | 82.4  | 80.9           | 89.2  | 13.4 | 15.2     | 9.7     | 237 | No  |  |
| 12  | 6   | 1050                  | 35   | 43.0            | 49.7                            | 47.5                              | 51.8  | 86.4  | 83.1           | 88.2  | 13.1 | 15.0     | 9.9     | 247 | No  |  |
| 13  | 7   | 980                   | 50   | 45.0            | 50.1                            | 47.8                              | 50.6  | 86.1  | 82.9           | 88.1  | 12.7 | 16.5     | 10.3    | 248 | No  |  |
| 14  | 8   | 1050                  | 10   | 0               | 31.5                            | 30.9                              | 32.9  | 55.2  | 52.9           | 59.5  | 28.9 | 29.1     | 26.9    | 151 | Yes |  |
| 15  | 9   | 900                   | 100  | 100             | 113.2                           | 110.9                             | 117.8 | 144.2 | 141.8          | 149.6 | 2.3  | 3.1      | 0.9     | 475 | No  |  |
| 16  | 1   | 750                   | 5    | 0               | 30.6                            | 30.2                              | 31.8  | 47.2  | 45.7           | 46.3  | 27.5 | 31.8     | 25.7    | 150 | Yes |  |
| 17  | 1   | 1000                  | 0.03 | 0               | 31.5                            | 30.8                              | 31.5  | 47.6  | 46.8           | 47.1  | 28.2 | 31.2     | 30.0    | 145 | Yes |  |
| 18  | 1   | —                     | —    | 0               | 85.2                            | 90.8                              | 100.4 | 88.7  | 95.2           | 103.2 | 2.5  | 1.1      | 0.6     | 270 | Yes |  |

Note:

(1) Example

(2) Steel

(3) L: longitudinal, D: diagonal, T: transverse

0.155% in excess of 0.15% and a (C+N) content of 0.22% in excess of 0.20 %, and thus, the product had a 100% martensitic structure after the continuous heat treatment, leading to a combination of great strength with poor elongation.

At the heating temperature of the continuous finish heat treatment (750° C.) used in Example 16, Steel 1 employed did not form a two-phase of ferrite and austenite. Accordingly, the product after the finish heat treatment had a single phase structure of ferrite, exhibiting a combination of high elongation with poor strength and hardness.

In Example 17, the cold rolled strip of Steel 1 was heated in a box furnace and allowed to cool in the same furnace at a cooling rate of 0.03° C./sec insufficient for transformation of the austenite to martensite. Accordingly, the product after the heat treatment contained no

These examples illustrate commercial production of low Cr 2CR materials according to the invention, using a continuous heat treatment furnace, 55

Steels having chemical compositions indicated in Table 9 were cast, hot rolled to a thickness of 3.6 mm, annealed at a temperature of 780° C. for 6 hours in a furnace, allowed to cool in the same furnace, pickled and cold rolled to a thickness of 0.3 mm under the conditions of cold rolling and intermediate annealing indicated in Table 10. Each cold rolled strip was continuously finish heat treated with a time of uniform heating of 1 minute in a continuous heat treatment furnace under conditions indicated in Table 10, except for in Examples 28 and 29. In Example 28 the cold rolled strip was heated in a box furnace with a time of uniform

EXAMPLE 19-29

heating of about 6 hours and allowed to cool in the same furnace. In Example 29, a hot rolled strip of Steel 11 of a thickness of 3.6 mm was annealed, pickled, cold rolled, air cooled and temper rolled to a thickness of 0.3 mm under conditions indicated in Table 10. The time of uniform heating in the intermediate annealing step was 1 minute in all Examples. Specimens of the products were tested for 0.2% proof stress, tensile strength and elongation in directions of 0° (longitudinal), 45° (diagonal) and 90° (transverse) to the direction of rolling, and for amount of martensite and hardness. On broken specimens from the tensile test, yes or no of ridging occurrence was observed. The results are shown in Table 10.

Examples 19-25 are in accordance with the invention, whereas Examples 26-29 are controls.

As seen from Table 10, steel strips of a duplex structure containing from about 55 to about 82% by volume of martensite having a combination of great strength and hardness as well as good elongation were obtained by processes of Examples 19-25 according to the invention. The products of the invention exhibited reduced plane anisotropy in respect of 0.2% proof stress, tensile strength and elongation.

In contrast, Steel 17 used in Example 26 had a (C+N) content as low as 0.012%, and in consequence, no martensite was formed by the continuous finish heat treatment. The product of Example 26 had poor strength and hardness.

At the heating temperature of the continuous finish heat treatment (800° C.) used in Example 27, Steel 11 employed did not form a two-phase of ferrite and austenite. Accordingly, the product after the finish heat treatment had a single phase structure of ferrite, exhibiting a combination of high elongation with poor strength and hardness.

In Example 28, the cold rolled strip of Steel 11 was heated in a box furnace and allowed to cool in the same furnace at a cooling rate of 0.03° C./sec insufficient for transformation of the austenite to martensite. Accordingly, the product after the heat treatment contained no martensite transformed, exhibiting a combination of high elongation with poor strength and hardness, as was the case in Example 27.

The product of Example 29 was a temper rolled material which had, when compared with the products of the invention, remarkably low elongation, high yield ratio (a ratio of 0.2% proof stress to tensile strength) and prominent plane anisotropy in respect of 0.2% proof stress, tensile strength and elongation. Apparently, such a product is inferior to the products of the invention regarding workability or formability and shape precision after worked or formed.

Table 10 further reveals that broken specimens from the tensile test of Examples 26, 27, 28 and 29 showed occurrence of ridging. In contrast the products of the invention were completely free from the problem of ridging. This means that the products of the invention work well in press-forming.

TABLE 9

| Steel | C     | Si   | Mn   | P     | S     | (in % by weight) |       |       |        |       |                    |
|-------|-------|------|------|-------|-------|------------------|-------|-------|--------|-------|--------------------|
|       |       |      |      |       |       | Ni               | Cr    | N     | Al     | O     | Others             |
| 10    | 0.023 | 0.43 | 0.31 | 0.023 | 0.005 | 0.15             | 10.85 | 0.015 | 0.008  | 0.009 |                    |
| 11    | 0.021 | 0.58 | 0.53 | 0.027 | 0.004 | 0.08             | 13.29 | 0.062 | 0.013  | 0.008 |                    |
| 12    | 0.083 | 0.54 | 0.45 | 0.018 | 0.006 | 0.16             | 12.08 | 0.009 | 0.150  | 0.007 |                    |
| 13    | 0.050 | 1.43 | 0.51 | 0.016 | 0.006 | 0.17             | 12.20 | 0.011 | 0.013  | 0.011 |                    |
| 14    | 0.043 | 0.52 | 0.39 | 0.018 | 0.005 | 0.21             | 13.51 | 0.009 | 0.009  | 0.007 | B 0.0023           |
| 15    | 0.040 | 0.45 | 0.51 | 0.019 | 0.006 | 0.10             | 12.57 | 0.009 | <0.005 | 0.014 | Mo 0.49            |
| 16    | 0.047 | 0.46 | 0.49 | 0.019 | 0.001 | 0.11             | 12.63 | 0.015 | <0.005 | 0.011 | REM 0.033, Y 0.025 |
| 17    | 0.006 | 0.41 | 0.30 | 0.020 | 0.007 | 0.12             | 12.11 | 0.006 | <0.005 | 0.009 |                    |

TABLE 10

| Ex. | St. | Conditions of cold rolling<br>(1) and annealing (3)                                                                 | tempera-<br>ture | Finish heat<br>treatment      |     | Amount of<br>martensite<br>(% by vol) | Properties (4) |      |      | Tensile<br>strength (kgf/mm <sup>2</sup> ) |      |       |
|-----|-----|---------------------------------------------------------------------------------------------------------------------|------------------|-------------------------------|-----|---------------------------------------|----------------|------|------|--------------------------------------------|------|-------|
|     |     |                                                                                                                     |                  | rate of<br>cooling<br>°C./sec | °C. |                                       | L              | D    | T    | L                                          | D    | T     |
| 19  | 10  | 3.6 <sup>t</sup> → CR → 1.0 <sup>t</sup> → An800° C. → CR → 0.3 <sup>t</sup> mm                                     | 1000             | 100                           |     | 81.6                                  | 66.2           | 68.4 | 69.0 | 95.2                                       | 97.5 | 98.8  |
| 20  | 11  | 3.6 <sup>t</sup> → CR → 1.0 <sup>t</sup> → An800° C. → CR → 0.3 <sup>t</sup> mm                                     | 1050             | 210                           |     | 77.6                                  | 67.4           | 69.7 | 70.2 | 96.8                                       | 99.2 | 101.3 |
| 21  | 12  | 3.6 <sup>t</sup> → CR → 1.8 <sup>t</sup> → An780° C. → CR → 0.9 <sup>t</sup> → An780° C. → CR → 0.3 <sup>t</sup> mm | 980              | 25                            |     | 68.8                                  | 55.0           | 55.4 | 55.8 | 83.0                                       | 85.6 | 84.3  |
| 22  | 13  | 3.6 <sup>t</sup> → CR → 1.0 <sup>t</sup> → An730° C → CR → 0.3 <sup>t</sup> mm                                      | 980              | 150                           |     | 62.5                                  | 59.3           | 60.5 | 59.7 | 93.1                                       | 95.8 | 95.4  |
| 23  | 14  | 3.6 <sup>t</sup> → CR → 1.8 <sup>t</sup> → An780° C. → CR → 0.9 <sup>t</sup> → An780° C. → CR → 0.3 <sup>t</sup> mm | 980              | 20                            |     | 57.5                                  | 47.7           | 52.8 | 49.3 | 79.8                                       | 83.2 | 81.5  |
| 24  | 15  | 3.6 <sup>t</sup> → CR → 1.0 <sup>t</sup> → An800° C. → CR → 0.3 <sup>t</sup> mm                                     | 1000             | 75                            |     | 66.6                                  | 54.7           | 55.2 | 55.5 | 83.2                                       | 84.8 | 84.5  |
| 25  | 16  | 3.6 <sup>t</sup> → CR → 1.0 <sup>t</sup> → An800° C. → CR → 0.3 <sup>t</sup> mm                                     | 950              | 75                            |     | 71.2                                  | 61.2           | 63.4 | 64.2 | 90.1                                       | 92.4 | 93.8  |
| 26  | 17  | 3.6 <sup>t</sup> → CR → 1.0 <sup>t</sup> → An780° C. → CR → 0.3 <sup>t</sup> mm                                     | 1050             | 10                            |     | 10.5                                  | 35.0           | 36.1 | 36.2 | 61.8                                       | 65.2 | 64.0  |
| 27  | 11  | 3.6 <sup>t</sup> → CR → 1.0 <sup>t</sup> → An800° C. → CR → 0.3 <sup>t</sup> mm                                     | 800              | 5                             |     | 0                                     | 30.5           | 31.1 | 29.6 | 45.7                                       | 47.1 | 46.3  |
| 28  | 11  | 3.6 <sup>t</sup> → CR → 1.0 <sup>t</sup> → An800° C. → CR → 0.3 <sup>t</sup> mm                                     | 1000             | 0.03                          |     | 0                                     | 31.2           | 31.0 | 30.2 | 46.2                                       | 47.6 | 47.0  |
| 29  | 11  | 3.6 <sup>t</sup> → CR → 1.2 <sup>t</sup> → An750° C. → CR → 0.3 <sup>t</sup> mm                                     | —                | —                             |     | 0                                     | 85.0           | 90.1 | 93.7 | 87.5                                       | 93.7 | 98.0  |

| Ex. | St. | Conditions of cold rolling<br>(1) and annealing (3)                                                                 | Properties (4) |          |         | (4) |
|-----|-----|---------------------------------------------------------------------------------------------------------------------|----------------|----------|---------|-----|
|     |     |                                                                                                                     | Elongation (%) | Hardness | Ridging |     |
| L   | D   | T                                                                                                                   | Hv             | (4)      |         |     |
| 19  | 10  | 3.6 <sup>t</sup> → CR → 1.0 <sup>t</sup> → An800° C. → CR → 0.3 <sup>t</sup> mm                                     | 11.2           | 9.6      | 9.8     | 293 |
| 20  | 11  | 3.6 <sup>t</sup> → CR → 1.0 <sup>t</sup> → An800° C. → CR → 0.3 <sup>t</sup> mm                                     | 10.1           | 9.2      | 9.4     | 311 |
| 21  | 12  | 3.6 <sup>t</sup> → CR → 1.8 <sup>t</sup> → An780° C. → CR → 0.9 <sup>t</sup> → An780° C. → CR → 0.3 <sup>t</sup> mm | 13.0           | 11.3     | 12.3    | 261 |
| 22  | 13  | 3.6 <sup>t</sup> → CR → 1.0 <sup>t</sup> → An730° C. → CR → 0.3 <sup>t</sup> mm                                     | 12.2           | 12.0     | 11.4    | 276 |
| 23  | 14  | 3.6 <sup>t</sup> → CR → 1.8 <sup>t</sup> → An780° C. → CR → 0.9 <sup>t</sup> → An780° C. → CR → 0.3 <sup>t</sup> mm | 15.0           | 13.6     | 14.3    | 236 |

TABLE 10-continued

| Steel | C  | Si               | Mn                                                             | P | S | Ni   | Cr   | N    | Al  | Properties (4) |           |
|-------|----|------------------|----------------------------------------------------------------|---|---|------|------|------|-----|----------------|-----------|
|       |    |                  |                                                                |   |   |      |      |      |     | rate of        | Amount of |
| 24    | 15 | 3.6 <sup>t</sup> | → CR → 1.0 <sup>t</sup> → An800° C. → CR → 0.3 <sup>t</sup> mm |   |   | 13.2 | 11.4 | 11.9 | 263 | No             |           |
| 25    | 16 | 3.6 <sup>t</sup> | → CR → 1.0 <sup>t</sup> → An800° C. → CR → 0.3 <sup>t</sup> mm |   |   | 11.4 | 9.7  | 9.8  | 294 | No             |           |
| 26    | 17 | 3.6 <sup>t</sup> | → CR → 1.0 <sup>t</sup> → An780° C. → CR → 0.3 <sup>t</sup> mm |   |   | 18.9 | 17.8 | 21.4 | 179 | Yes            |           |
| 27    | 11 | 3.6 <sup>t</sup> | → CR → 1.0 <sup>t</sup> → An800° C. → CR → 0.3 <sup>t</sup> mm |   |   | 31.6 | 27.5 | 29.5 | 142 | Yes            |           |
| 28    | 11 | 3.6 <sup>t</sup> | → CR → 1.0 <sup>t</sup> → An800° C. → CR → 0.3 <sup>t</sup> mm |   |   | 30.2 | 28.2 | 30.5 | 145 | Yes            |           |
| 29    | 11 | 3.6 <sup>t</sup> | → CR → 1.2 <sup>t</sup> → An750° C. → CR → 0.3 <sup>t</sup> mm |   |   | 2.6  | 1.2  | 0.7  | 270 | Yes            |           |

Note:

(1) Example

(2) Steel

(3) t; thickness(mm), CR; cold rolling, An; annealing

(4) L; longitudinal, D; diagonal, T; transverse

## EXAMPLE 30-40

These examples illustrate commercial production of high Cr 2CR materials according to the invention, using a continuous heat treatment furnace,

Steels having chemical compositions indicated in Table 11 were cast, hot rolled to a thickness of 3.6 mm, annealed at a temperature of 780° C. for 6 hours in a furnace, allowed to cool in the same furnace, pickled and cold rolled to a thickness of 0.3 mm under the conditions of cold rolling and intermediate annealing indicated in Table 12. Each cold rolled strip was continuously finish heat treated with a time of uniform heating of 1 minute in a continuous heat treatment furnace under conditions indicated in Table 12, except for in Examples 39 and 40. In Example 39 the cold rolled strip was heated in a box furnace with a time of uniform heating of about 6 hours and allowed to cool in the same furnace. In Example 40, a hot rolled strip of Steel 19 of a thickness of 3.6 mm was annealed, pickled, cold rolled, air cooled and temper rolled to a thickness of 0.3 mm under conditions indicated in Table 12. The time of uniform heating in the intermediate annealing step 1 minute in all Examples. Specimens of the products were tested for 0.2% proof stress, tensile strength and elongation in directions of 0° (longitudinal), 45° (diagonal) and 90° (transverse) to the direction of rolling, and for amount of martensite and hardness. On broken specimens from the tensile test, yes or no of ridging occurrence was observed. The results are shown in Table 12.

Examples 30-36 are in accordance with the invention, whereas Examples 37-40 are controls.

As seen from Table 12, steel strips of a duplex structure containing from about 30 to about 60% by volume of martensite having a combination of great strength and hardness as well as good elongation were obtained by processes of Examples 30-36 according to the invention,

15 plane anisotropy in respect of 0.2% proof stress, tensile strength and elongation.

In contrast, Steel 25 used in Example 37 had a carbon content of 0.155% and a (C+N) content of 0.220%, which were unduly high, and thus, the product had a 100% martensitic structure after the continuous heat treatment, leading to a combination of great strength with poor elongation.

20 At the heating temperature of the continuous finish heat treatment (780° C.) used in Example 38, Steel 19 employed did not form a two-phase of ferrite and austenite. Accordingly, the product after the finish heat treatment had a single phase structure of ferrite, exhibiting a combination of high elongation with poor strength and hardness.

25 In Example 39, the cold rolled strip of Steel 19 was heated in a box furnace and allowed to cool in the same furnace at a cooling rate of 0.03° C./sec insufficient for transformation of the austenite to martensite. Accordingly, the product after the heat treatment contained no martensite transformed, exhibiting a combination of high elongation with poor strength and hardness.

30 The product of Example 40 was a temper rolled material which had, when compared with the products of the invention, remarkably low elongation, high yield ratio (a ratio of 0.2% proof stress to tensile strength) and prominent plane anisotropy in respect of 0.2% proof stress, tensile strength and elongation. Apparently, such a product is inferior to the products of the invention regarding workability or formability and shape precision after worked or formed.

35 45 50 55 Table 12 further reveals that broken specimens from the tensile test of Examples 38-40 showed occurrence of ridging. In contrast the products of the invention were completely free from the problem of ridging. This means that the products of the invention work well in press-forming.

TABLE 11

| Steel | C     | Si   | Mn   | P     | S     | (in % by weight) |       |       |        |       |                    |
|-------|-------|------|------|-------|-------|------------------|-------|-------|--------|-------|--------------------|
|       |       |      |      |       |       | Ni               | Cr    | N     | Al     | O     | Others             |
| 18    | 0.055 | 0.43 | 0.45 | 0.021 | 0.005 | 0.12             | 15.05 | 0.041 | 0.022  | 0.008 |                    |
| 19    | 0.068 | 0.46 | 0.40 | 0.018 | 0.006 | 0.09             | 16.44 | 0.022 | <0.005 | 0.018 |                    |
| 20    | 0.116 | 0.41 | 0.60 | 0.022 | 0.006 | 0.12             | 18.21 | 0.013 | 0.018  | 0.008 |                    |
| 21    | 0.086 | 1.49 | 0.29 | 0.018 | 0.006 | 0.17             | 16.59 | 0.033 | 0.005  | 0.012 |                    |
| 22    | 0.048 | 0.44 | 0.48 | 0.021 | 0.006 | 0.11             | 16.53 | 0.059 | <0.005 | 0.016 | B 0.0017           |
| 23    | 0.035 | 0.46 | 0.53 | 0.021 | 0.005 | 0.12             | 16.38 | 0.104 | 0.130  | 0.006 | Mo 0.55            |
| 24    | 0.075 | 0.45 | 0.51 | 0.018 | 0.001 | 0.12             | 16.48 | 0.028 | 0.018  | 0.010 | REM 0.025, Y 0.031 |
| 25    | 0.155 | 0.63 | 0.45 | 0.021 | 0.005 | 0.10             | 14.31 | 0.065 | 0.027  | 0.015 |                    |

tion. The products of the invention exhibited reduced

TABLE 12

| Finish heat treatment | Properties (4) |           |            | Tensile strength |
|-----------------------|----------------|-----------|------------|------------------|
|                       | rate of        | Amount of | 0.2% proof |                  |

TABLE 12-continued

| Ex. | St. | Conditions of cold rolling<br>(1) (2) and annealing (3)                                                             | temperature<br>°C. | cooling<br>°C./sec | martensite<br>(% by vol) | (kgf/mm <sup>2</sup> ) |       |       | (kgf/mm <sup>2</sup> ) |  |
|-----|-----|---------------------------------------------------------------------------------------------------------------------|--------------------|--------------------|--------------------------|------------------------|-------|-------|------------------------|--|
|     |     |                                                                                                                     |                    |                    |                          | L                      | D     | T     | L                      |  |
| 30  | 18  | 3.6 <sup>t</sup> → CR → 1.0 <sup>t</sup> → An730° C. → CR → 0.3 <sup>t</sup> mm                                     | 1050               | 100                | 58.7                     | 60.5                   | 60.3  | 58.7  | 90.9                   |  |
| 31  | 19  | 3.6 <sup>t</sup> → CR → 1.0 <sup>t</sup> → An730° C. → CR → 0.3 <sup>t</sup> mm                                     | 1000               | 10                 | 36.5                     | 40.3                   | 41.3  | 40.8  | 76.7                   |  |
| 32  | 20  | 3.6 <sup>t</sup> → CR → 1.8 <sup>t</sup> → An730° C. → CR → 0.9 <sup>t</sup> → An730° C. → CR → 0.3 <sup>t</sup> mm | 950                | 6                  | 39.0                     | 48.3                   | 49.1  | 48.2  | 84.7                   |  |
| 33  | 21  | 3.6 <sup>t</sup> → CR → 1.0 <sup>t</sup> → An720° C. → CR → 0.3 <sup>t</sup> mm                                     | 1050               | 150                | 30.5                     | 42.5                   | 43.9  | 44.5  | 89.6                   |  |
| 34  | 22  | 3.6 <sup>t</sup> → CR → 1.8 <sup>t</sup> → An730° C. → CR → 0.9 <sup>t</sup> → An730° C. → CR → 0.3 <sup>t</sup> mm | 980                | 25                 | 46.1                     | 51.8                   | 52.6  | 51.7  | 86.5                   |  |
| 35  | 23  | 3.6 <sup>t</sup> → CR → 1.0 <sup>t</sup> → An750° C. → CR → 0.3 <sup>t</sup> mm                                     | 1050               | 35                 | 43.0                     | 49.1                   | 50.2  | 49.3  | 85.0                   |  |
| 36  | 24  | 3.6 <sup>t</sup> → CR → 1.0 <sup>t</sup> → An750° C. → CR → 0.3 <sup>t</sup> mm                                     | 1000               | 50                 | 45.0                     | 50.3                   | 51.5  | 51.1  | 86.1                   |  |
| 37  | 25  | 3.6 <sup>t</sup> → CR → 1.0 <sup>t</sup> → An800° C. → CR → 0.3 <sup>t</sup> mm                                     | 900                | 100                | 100                      | 112.5                  | 111.8 | 109.2 | 143.3                  |  |
| 38  | 19  | 3.6 <sup>t</sup> → CR → 1.0 <sup>t</sup> → An730° C. → CR → 0.3 <sup>t</sup> mm                                     | 780                | 10                 | 0                        | 33.4                   | 35.5  | 34.0  | 51.6                   |  |
| 39  | 19  | 3.6 <sup>t</sup> → CR → 1.0 <sup>t</sup> → An730° C. → CR → 0.3 <sup>t</sup> mm                                     | 1000               | 0.03               | 0                        | 33.6                   | 35.8  | 34.1  | 52.9                   |  |
| 40  | 19  | 3.6 <sup>t</sup> → CR → 1.2 <sup>t</sup> → An750° C. → CR → 0.3 <sup>t</sup> mm                                     | —                  | —                  | 0                        | 86.5                   | 91.7  | 99.1  | 89.3                   |  |

  

| Ex. | St. | Conditions of cold rolling<br>(1) (2) and annealing (3)                                                             | Properties (4)                             |       |                |      |          |     |         |
|-----|-----|---------------------------------------------------------------------------------------------------------------------|--------------------------------------------|-------|----------------|------|----------|-----|---------|
|     |     |                                                                                                                     | Tensile strength<br>(kgf/mm <sup>2</sup> ) |       | Elongation (%) |      | Hardness |     | Ridging |
| (D) | (T) | (L)                                                                                                                 | (D)                                        | (T)   | (HV)           | (4)  |          |     |         |
| 30  | 18  | 3.6 <sup>t</sup> → CR → 1.0 <sup>t</sup> → An730° C. → CR → 0.3 <sup>t</sup> mm                                     | 91.6                                       | 91.3  | 11.3           | 12.8 | 11.2     | 280 | No      |
| 31  | 19  | 3.6 <sup>t</sup> → CR → 1.0 <sup>t</sup> → An730° C. → CR → 0.3 <sup>t</sup> mm                                     | 79.2                                       | 77.3  | 16.2           | 15.3 | 17.6     | 223 | No      |
| 32  | 20  | 3.6 <sup>t</sup> → CR → 1.8 <sup>t</sup> → An730° C. → CR → 0.9 <sup>t</sup> → An730° C. → CR → 0.3 <sup>t</sup> mm | 86.1                                       | 85.1  | 14.7           | 14.2 | 15.1     | 256 | No      |
| 33  | 21  | 3.6 <sup>t</sup> → CR → 1.0 <sup>t</sup> → An720° C. → CR → 0.3 <sup>t</sup> mm                                     | 89.9                                       | 88.4  | 13.8           | 13.7 | 13.0     | 246 | No      |
| 34  | 22  | 3.6 <sup>t</sup> → CR → 1.8 <sup>t</sup> → An730° C. → CR → 0.9 <sup>t</sup> → An730° C. → CR → 0.3 <sup>t</sup> mm | 87.2                                       | 88.0  | 13.2           | 12.8 | 13.5     | 262 | No      |
| 35  | 23  | 3.6 <sup>t</sup> → CR → 1.0 <sup>t</sup> → An750° C. → CR → 0.3 <sup>t</sup> mm                                     | 86.6                                       | 85.0  | 14.5           | 13.9 | 14.9     | 246 | No      |
| 36  | 24  | 3.6 <sup>t</sup> → CR → 1.0 <sup>t</sup> → An750° C. → CR → 0.3 <sup>t</sup> mm                                     | 86.9                                       | 87.5  | 14.1           | 13.2 | 15.1     | 248 | No      |
| 37  | 25  | 3.6 <sup>t</sup> → CR → 1.0 <sup>t</sup> → An800° C. → CR → 0.3 <sup>t</sup> mm                                     | 145.2                                      | 147.4 | 2.8            | 1.9  | 1.1      | 472 | No      |
| 38  | 19  | 3.6 <sup>t</sup> → CR → 1.0 <sup>t</sup> → An730° C. → CR → 0.3 <sup>t</sup> mm                                     | 54.5                                       | 52.2  | 30.8           | 27.8 | 31.3     | 151 | Yes     |
| 39  | 19  | 3.6 <sup>t</sup> → CR → 1.0 <sup>t</sup> → An730° C. → CR → 0.3 <sup>t</sup> mm                                     | 56.1                                       | 52.4  | 29.9           | 25.8 | 30.1     | 153 | Yes     |
| 40  | 19  | 3.6 <sup>t</sup> → CR → 1.2 <sup>t</sup> → An750° C. → CR → 0.3 <sup>t</sup> mm                                     | 95.1                                       | 104.0 | 2.7            | 1.5  | 0.7      | 265 | Yes     |

Note:

(1) Example

(2) Steel

(3) t: thickness (mm), CR: cold rolling, An: annealing

(4) L: longitudinal, D: diagonal, T: transverse

## What is claimed is:

1. A process for the production of a strip of a chromium stainless steel of a duplex structure, consisting essentially of ferrite and martensite, having high strength and elongation as well as reduced plane anisotropy and having a hardness of at least HV 200, which process comprises:

a step of hot rolling a slab of a steel to provide a hot rolled strip, said steel comprising, by weight, from 10.0% to 20.0% of Cr, up to 0.15% of C, up to 0.12% of N, the (C+N) being not less than 0.02% but not more than 0.20%, up to 2.0% of Si, up to 1.0% of Mn and up to 0.6% of Ni, the balance being Fe and unavoidable impurities;

a step of cold rolling the hot rolled strip to provide a cold rolled strip of a desired thickness; and

a step of continuous final heat treatment in which the cold rolled strip is continuously passed through a heating zone where it is heated to a temperature ranging from the Ac1 point of the steel to 1100° C. to form a two-phase of ferrite and austenite and maintained at that temperature for not longer than 10 minutes, and the heated strip is cooled at a cooling rate sufficient to transform the austenite to martensite.

2. The process in accordance with claim 1 wherein in said continuous heat treatment step the cold rolled strip is heated to a temperature ranging from at least 100° C. above the Ac1 point of the steel to 1100° C. to form a two-phase of ferrite and austenite.

3. The process in accordance with claim 1 wherein in said continuous heat treatment step the cold rolled strip

is heated to a temperature ranging from 900° C. to 1100° C. to form a two-phase of ferrite and austenite.

4. The process in accordance with claim 1 wherein in said steel employed consists essentially of, by weight:

up to 0.10% of C,  
up to 2.0% of Si,  
up to 1.0% of Mn,  
up to 0.040% of P,  
up to 0.030% of S,  
up to 0.60% of Ni,  
from 10.0% to 14.0% of Cr,  
up to 0.08% of N, the (C+N) being not less than 0.02% but not more than 0.12%,  
up to 0.02% of O,  
up to 0.20% of Al,  
up to 0.0050% of B,  
up to 2.5% of Mo,  
up to 0.10% of REM, and  
up to 0.20% of Y, the balance being Fe and unavoidable impurities.

5. The process in accordance with claim 1 wherein in said steel employed consists essentially of, by weight:

up to 0.15% of C,  
up to 2.0% of Si,  
up to 1.0% of Mn,  
up to 0.040% of P,  
up to 0.030% of S,  
up to 0.60% of Ni,  
more than 14.0% to 20.0% of Cr,  
up to 0.12% of N, the (C+N) being not less than 0.03% but not more than 0.20%,  
up to 0.02% of O,  
up to 0.20% of Al,

up to 0.0050% of B,  
up to 2.5% of Mo,  
up to 0.10% of REM, and  
up to 0.20% of Y, the balance being Fe and unavoidable impurities.

6. A process for the production of a strip of a chromium stainless steel of a duplex structure, consisting essentially of ferrite and martensite, having high strength and elongation as well as reduced plane anisotropy and having a hardness of at least HV 200, which process comprises:

a step of hot rolling a slab of a steel to provide a hot rolled strip, said steel consisting essentially of, by weight:

up to 0.10% of C,  
up to 2.0% of Si,  
up to 1.0% of Mn,  
up to 0.040% of P,  
up to 0.030% of S,  
up to 0.60% of Ni,  
from 10.0% to 14.0% of Cr,  
up to 0.08% of N, the (C+N) being not less than 0.02% but not more than 0.12%,  
up to 0.02% of O,  
up to 0.20% of Al,  
up to 0.0050% of B,  
up to 2.5% of Mo,  
up to 0.10% of REM, and  
up to 0.20% of Y, the balance being Fe and unavoidable impurities;

at least two steps of cold rolling the hot rolled strip to provide a cold rolled strip of a desired thickness, including a step of intermediate annealing between the successive two cold rolling steps, said intermediate annealing comprising heating and maintaining the strip at a temperature to form a single phase of ferrite; and

a step of continuous final heat treatment in which the cold rolled strip is continuously passed through a heating zone where it is heated to a temperature ranging from the Ac1 point of the steel to 1100° C. to form a two-phase of ferrite and austenite and maintained at that temperature for not longer than 10 minutes, and the heated strip is cooled at a cooling rate sufficient to transform the austenite to martensite.

7. The process in accordance with claim 6 wherein in said continuous heat treatment step the cold rolled strip is heated to a temperature ranging from at least 100° C. above the Ac1 point of the steel to 1100° C. to form a two-phase of ferrite and austenite.

8. The process in accordance with claim 6 wherein in said continuous heat treatment step the cold rolled strip

is heated to a temperature ranging from 900° C. to 1100° C. to form a two-phase of ferrite and austenite.

9. A process for the production of a strip of a chromium stainless steel of a duplex structure, consisting essentially of ferrite and martensite, having high strength and elongation as well as reduced plane anisotropy and having a hardness of at least HV 200, which process comprises:

a step of hot rolling a slab of a steel to provide a hot rolled strip, said steel consisting essentially of, by weight:

up to 0.15% of C,  
up to 2.0% of Si,  
up to 1.0% of Mn,  
up to 0.040% of P,  
up to 0.030% of S,  
up to 0.60% of Ni,  
more than 14.0% to 20.0% of Cr,  
up to 0.12% of N, the (C+N) being not less than 0.03% but not more than 0.20%,  
up to 0.02% of O,  
up to 0.20% of Al,  
up to 0.0050% of B,  
up to 2.5% of Mo,

up to 0.10% of REM, and  
up to 0.20% of Y, the balance being Fe and unavoidable impurities;

at least two steps of cold rolling the hot rolled strip to provide a cold rolled strip of a desired thickness, including a step of intermediate annealing between the successive two cold rolling steps, said intermediate annealing comprising heating and maintaining the strip at a temperature to form a single phase of ferrite; and

a step of continuous final heat treatment in which the cold rolled strip is continuously passed through a heating zone where it is heated to a temperature ranging from the Ac1 point of the steel to 1100° C. to form a two-phase of ferrite and austenite and maintained at that temperature for not longer than 10 minutes, and the heated strip is cooled at a cooling rate sufficient to transform the austenite to martensite.

10. The process in accordance with claim 9 wherein in said continuous heat treatment step the cold rolled strip is heated to a temperature ranging from at least 100° C. above the Ac1 point of the steel to 1100° C. to form a two-phase of ferrite and austenite.

11. The process in accordance with claim 9 wherein in said continuous heat treatment step the cold rolled strip is heated to a temperature ranging from 900° to 1100° C. to form a two-phase of ferrite and austenite.

\* \* \* \* \*



US004812176B1

## REEXAMINATION CERTIFICATE (2836th)

United States Patent [19]

Tanaka et al.

[45] Certificate Issued Apr. 9, 1996

[11] B1 4,812,176

[54] **PROCESS FOR THE PRODUCTION OF A STRIP OF A CHROMIUM STAINLESS STEEL OF A DUPLEX STRUCTURE HAVING HIGH STRENGTH AND ELONGATION AS WELL AS REDUCED PLANE ANISOTROPY**

[75] Inventors: **Teruo Tanaka; Katsuhisa Miyakusu; Hiroshi Fujimoto**, all of Yamaguchi, Japan

[73] Assignee: **Nissin Steel Co., Ltd.**, Tokyo, Japan

**Reexamination Request:**  
No. 90/003,605, Oct. 17, 1994

**Reexamination Certificate for:**

Patent No.: **4,812,176**  
Issued: **Mar. 14, 1989**  
Appl. No.: **134,874**  
Filed: **Dec. 18, 1987**

[51] Int. Cl.<sup>6</sup> ..... **C21D 8/02**  
[52] U.S. Cl. ..... **148/597; 148/610**  
[58] Field of Search ..... **148/605, 610, 148/599, 597**

[56] **References Cited**

## U.S. PATENT DOCUMENTS

2,145,171 1/1939 Giles .  
3,309,238 3/1967 Randak et al. .  
3,650,848 3/1972 Schneider et al. .  
3,674,467 7/1972 Chalk .  
3,861,909 1/1975 Caton .  
3,989,514 11/1976 Fujioka et al. .  
4,049,430 9/1977 Myers .  
4,141,762 2/1979 Yamaguchi et al. .  
4,564,392 1/1986 Ohhashi et al. .

## FOREIGN PATENT DOCUMENTS

1951908 8/1971 Germany .  
2023657 6/1979 United Kingdom .

## OTHER PUBLICATIONS

*The Making, Shaping and Treating of Steel* (10th ed. 1985), pp. 1100, 1264, 1335.

Peckner and Bernstein, *Handbook of Stainless Steels* (McGraw-Hill 1977) p. 14-2.

FIG. IV-2 of *Stainless Steel Fabrication* (Allegheny Ludlum Corp. 1959), p. 132.

"Effects of Alloying Elements And Heat Treatment On Microstructures And Mechanical Properties Of Ferrite-Martensite Dual Phase Stainless Steel Sheets" Miyakusu et al. (of Nissin Steel Co., Ltd.) *Proceedings of International Conference on Stainless Steels*, 1991, Chiba, ISIJ.

"Anisotropy in Metals", Chalmers, *Progress in Metal Physics* 2 (Interscience publishers 1950), p. 115.

"Anisotropy in Polycrystalline Materials", Honeycombe, *The Plastic Deformation of Metals* (2d ed., Edward Arnold/American Society for Metals 1984), pp. 326-327.

**Primary Examiner**—Deborah Yee

[57] **ABSTRACT**

Process for producing steel strip of duplex structure wherein cold rolled strip of chromium stainless steel comprising, in addition to Fe, 10.0% to 20.0% of Cr, to 0.15% of C, to 0.12% of N, the (C+N) being 0.02% to 0.20%, to 2.0% of Si, to 1.0% of Mn and to 0.6% of Ni, is continuously passed through a heating zone where it is heated to form a two-phase of ferrite and austenite and the heated strip is cooled at a cooling rate sufficient to transform the austenite to martensite. The product has high strength and elongation reduced plane anisotropy and hardness of at least HV 200.



**REEXAMINATION CERTIFICATE  
ISSUED UNDER 35 U.S.C. 307**

THE PATENT IS HEREBY AMENDED AS  
INDICATED BELOW.

Matter enclosed in heavy brackets [ ] appeared in the patent, but has been deleted and is no longer a part of the patent; matter printed in italics indicates additions made to the patent.

AS A RESULT OF REEXAMINATION, IT HAS BEEN DETERMINED THAT:

Claims 1-11 are cancelled.

New claims 12-16 are added and determined to be patentable.

12. *A process for the production of a strip of a chromium stainless steel of a duplex structure, consisting essentially of ferrite and martensite, having high strength and elongation as well as reduced plane anisotropy and having a hardness of at least HV 200, which process comprises:*

a) *hot rolling a slab of a steel to provide a hot rolled strip, said steel comprising, by weight, from 10.0% to 20.0% of Cr, up to 0.15% of C, up to 0.12% of N, the (C+N) being not less than 0.02% but not more than 0.20%, up to 2.0% of Si, up to 1.0% of Mn and up to 0.6% of Ni, the balance being Fe and unavoidable impurities;*

b) *cold rolling the hot rolled strip to provide a cold rolled strip of a desired thickness; and*

c) *continuous finish heat treatment in which the cold rolled strip is continuously passed through a heating zone where it is heated to a temperature ranging from at least 100° C. above the Ac<sub>1</sub> point of the steel to 1100° C. to form a two-phase of ferrite and austenite and maintained at that temperature for not longer than 10 minutes, and the heated strip is cooled at a cooling rate sufficient to transform the austenite to martensite.*

13. *The process in accordance with claim 12 wherein in said steel employed consists essentially of, by weight:*

*up to 0.10% of C,*

*up to 2.0% of Si,*

*up to 1.0% of Mn,*

*up to 0.040% of P,*

*up to 0.030% of S,*

*up to 0.60% of Ni,*

*from 10.0% to 14.0% Cr,*

*up to 0.08% of N, the (C+N) being not less than 0.02% but not more than 0.12%,*

*up to 0.02% of O,*

*up to 0.20% of Al,*

*up to 0.0050% of B,*

*up to 2.5% of Mo,*

*up to 0.10% of REM, and*

*up to 0.20% of Y,*

*the balance being Fe and unavoidable impurities.*

14. *The process in accordance with claim 12 wherein in said steel employed consists essentially of, by weight:*

*up to 0.15% of C,*

*up to 2.0% of Si,*

*up to 1.0% of Mn,*  
*up to 0.040% of P,*  
*up to 0.030% of S,*  
*up to 0.60% of Ni,*

*more than 14.0% to 20.0% of Cr,*

*up to 0.12% of N, the (C+N) being not less than 0.03% but not more than 0.20%,*

*up to 0.02% of O,*

*up to 0.20% of Al,*

*up to 0.050% of B,*

*up to 2.5% of Mo,*

*up to 0.10% of REM, and*

*up to 0.20% of Y,*

*the balance being Fe and unavoidable impurities.*

15. *A process for the production of a strip of a chromium stainless steel of a duplex structure, consisting essentially of ferrite and martensite, having high strength and elongation as well as reduced plane anisotropy and having a hardness of at least HV 200, which process comprises:*

*a) hot rolling a slab of steel to provide a hot rolled strip, said steel consisting essentially of, by weight:*

*up to 0.10% of C,*

*up to 2.0% of Si,*

*up to 1.0% of Mn,*

*up to 0.040% of P,*

*up to 0.030% of S,*

*up to 0.60% of Ni,*

*from 10.0% to 14.0% of Cr,*

*up to 0.08% of N, the (C+N) being not less than 0.02% but not more than 0.12%,*

*up to 0.02% of O,*

*up to 0.20% of Al,*

*up to 0.0050% of B,*

*up to 2.5% of Mo,*

*up to 0.10% of REM, and*

*up to 0.20% of Y,*

*the balance being Fe and unavoidable impurities;*

*b) at least two steps of cold rolling the hot rolled strip to provide a cold rolled strip of a desired thickness, including a step of intermediate annealing between the successive two cold rolling steps, said intermediate annealing comprising heating and maintaining the strip at a temperature to form a single phase of ferrite; and*

*c) continuous finish heat treatment in which the cold rolled strip is continuously passed through a heating zone where it is heated to a temperature ranging from at least 100° C. above the Ac<sub>1</sub> point of the steel to 1100° C. to form a two-phase of ferrite and austenite and maintained at that temperature for not longer than 10 minutes, and the heated strip is cooled at a cooling rate sufficient to transform the austenite to martensite.*

16. *A process for the production of a strip of a chromium stainless steel of a duplex structure, consisting essentially of ferrite and martensite, having high strength and elongation as well as reduced plane anisotropy and having a hardness of at least HV 200, which process comprises:*

*a) hot rolling a slab of steel to provide a hot rolled strip, said steel consisting essentially of, by weight:*

*up to 0.15% of C,*

*up to 2.0% of Si,*

up to 1.0% of Mn,  
 up to 0.040% of P,  
 up to 0.030% of S,  
 up to 0.60% of Ni,  
 more than 14.0% to 20.0% of Cr,  
 up to 0.12% of N, the (C+N) being not less than 0.03% but  
 not more than 0.20%,  
 up to 0.02% of O,  
 up to 0.20% of Al,  
 up to 0.0050% of B,  
 up to 2.5% of Mo,  
 up to 0.10% of REM, and  
 up to 0.20% of Y,  
 the balance being Fe and unavoidable impurities;

5

10

15

b) at least two steps of cold rolling the hot rolled strip to provide a cold rolled strip of a desired thickness, including a step of intermediate annealing between the successive two cold rolling steps, said intermediate annealing comprising heating and maintaining the strip at a temperature to form a single phase of ferrite; and  
 c) a continuous finish heat treatment in which the cold rolled strip is continuously passed through a heating zone where it is heated to a temperature ranging from at least 100° C. above the  $A_{c1}$  point of the steel to 1100° C. to form a two-phase of ferrite and austenite and maintained at that temperature for not longer than 10 minutes, and the heated strip is cooled at a cooling rate sufficient to transform the austenite to martensite.

\* \* \* \* \*